



US009580866B2

(12) **United States Patent**  
**Brungardt**

(10) **Patent No.:** **US 9,580,866 B2**  
(b4) **Date of Patent:** **Feb. 28, 2017**

(54) **CATIONIC WET STRENGTH RESIN  
MODIFIED PIGMENTS IN WATER-BASED  
LATEX COATING APPLICATIONS**

(75) Inventor: **Clement L. Brungardt**, Oxford, PA  
(US)

(73) Assignee: **Solenis Technologies, L.P.** (CH)

(\*) Notice: Subject to any disclaimer, the term of this patent is extended or adjusted under 35 U.S.C. 154(b) by 0 days.

(21) Appl. No.: **12/789,918**

(22) Filed: **May 28, 2010**

(65) **Prior Publication Data**

US 2010/0310883 A1 Dec. 9, 2010

**Related U.S. Application Data**

(63) Continuation-in-part of application No. 12/477,432, filed on Jun. 3, 2009.

(51) **Int. Cl.**

**B05D 3/02** (2006.01)  
**D21H 19/36** (2006.01)  
**D21H 17/46** (2006.01)  
**D21H 17/52** (2006.01)  
**D21H 17/56** (2006.01)  
**D21H 19/40** (2006.01)  
**D21H 19/62** (2006.01)  
**D21H 19/80** (2006.01)  
**D21H 19/82** (2006.01)  
**D21H 21/20** (2006.01)  
**D21H 27/10** (2006.01)

(52) **U.S. Cl.**

CPC ..... **D21H 19/36** (2013.01); **D21H 17/46** (2013.01); **D21H 17/52** (2013.01); **D21H 17/56** (2013.01); **D21H 19/40** (2013.01); **D21H 19/62** (2013.01); **D21H 19/80** (2013.01); **D21H 19/822** (2013.01); **D21H 21/20** (2013.01); **D21H 27/10** (2013.01); Y10T 428/31587 (2015.04); Y10T 428/31591 (2015.04)

(58) **Field of Classification Search**

CPC ..... D21H 19/36; D21H 17/46; D21H 17/52; D21H 17/56; D21H 19/40; D21H 19/62; D21H 19/80; D21H 19/822; D21H 21/20; D21H 27/10; Y10T 428/31587; Y10T 428/31591

USPC ..... 427/391  
See application file for complete search history.

(56) **References Cited**

U.S. PATENT DOCUMENTS

2,795,545 A 6/1957 Gluesenkamp  
4,885,330 A 12/1989 Brungardt et al.

|                   |         |                               |
|-------------------|---------|-------------------------------|
| 5,169,441 A       | 12/1992 | Lauzon                        |
| 5,384,013 A *     | 1/1995  | Husband et al. .... 162/168.1 |
| 5,531,863 A       | 7/1996  | Propst                        |
| 5,668,246 A *     | 9/1997  | Maslanka ..... 528/336        |
| 5,885,340 A *     | 3/1999  | Bailey et al. .... 106/209.1  |
| 5,916,420 A       | 6/1999  | Wurster                       |
| 6,030,443 A       | 2/2000  | Bock et al.                   |
| 6,358,576 B1      | 3/2002  | Adur et al.                   |
| 6,359,040 B1      | 3/2002  | Burdick                       |
| 6,429,253 B1      | 8/2002  | Guerro et al.                 |
| 6,531,196 B1      | 3/2003  | Aho et al.                    |
| 6,554,961 B1      | 4/2003  | Riehle et al.                 |
| 6,722,560 B2      | 4/2004  | Player et al.                 |
| 7,081,512 B2      | 7/2006  | Riehle                        |
| 7,148,271 B2      | 12/2006 | Michelman et al.              |
| 7,150,522 B2 *    | 12/2006 | Sen ..... 347/101             |
| 2003/0199629 A1 * | 10/2003 | Gelman et al. ..... 524/514   |

FOREIGN PATENT DOCUMENTS

|    |            |         |
|----|------------|---------|
| WO | 0163049    | 8/2001  |
| WO | 2004099321 | 11/2004 |

OTHER PUBLICATIONS

F. Wu, "High Performance Tale for Barrier Packaging," 2007 TAPPI Coating and Graphic Arts Conference, (Miami) Apr. 22-25, 2007.  
M. Kleebauer, "Polymer Dispersions with Inorganic Pigments as a Back Barrier Coating on Folding Boxboard," 6th International Paper and coating Chemistry Symposium (Stockholm), Jun. 7-9, 2006.  
R. Popil, "Optimizing Water Resistance of Polymeric/pigmented Linerboard Coatings Using Pigments for Linerboard Wax Replacement," TAPPI—Paper Coatings and Graphic Arts Conference Proceedings, (Atlanta) Apr. 24-27, 2006.  
International Search Report and Written Opinion mailed Aug. 12, 2010.

\* cited by examiner

*Primary Examiner* — Robert S Walters, Jr.

(74) *Attorney, Agent, or Firm* — Joanne Rossi; Michael Herman

(57) **ABSTRACT**

Methods for improving one or more surface properties of a sheet of paper or paperboard, which method comprises (a) coating at least one side of the sheet of paper or paperboard with a dispersion having a cationic zeta potential formed by combining (1) a mixture containing one or more anionic pigments with (2) one or more polyamine-epihalohydrin cationic wet strength resins at a coating weight of from about 0.1 g/m<sup>2</sup> to about 20 g/m<sup>2</sup>; (b) drying the coated sheet of paper or paperboard; (c) applying a functional barrier top coating that resists one or more of the following: liquid water, water vapor, gas permeability, oil and grease, slip, and static or an anionic latex based pigment coating that imparts improved opacity, brightness, or printability. The invention also includes the dispersions as well as paper or paperboard coated with the dispersion.

**12 Claims, No Drawings**

**CATIONIC WET STRENGTH RESIN  
MODIFIED PIGMENTS IN WATER-BASED  
LATEX COATING APPLICATIONS**

This application is related to and claims the benefit of U.S. patent application Ser. No. 12/477,432, filed May 28, 2010.

**BACKGROUND OF THE INVENTION**

Paper board is widely used throughout the world in packaging applications. Paper board can be printed and folded into attractive and functional containers that are inexpensive, protect their contents, and are based on renewable and recyclable raw materials. Paperboard's poor barrier properties limit its usefulness in food packaging, especially in applications that require high barrier resistance to liquid water, water vapor, gas permeability, oil and grease, slip, and static. To overcome this limitation, others have added additional functional layers to the paperboard, thus increasing the paperboard's barrier properties. For example, laminated films, extruded polymer coatings, and wax coatings are known to improve paperboard's resistance to both liquid water and water vapor. These coatings require additional processing, are expensive relative to the cost of the untreated paperboard, and make the paperboard harder to recycle.

Recently, however, recyclable water-based latex barrier coatings have become available that improve paperboard's barrier properties while maintaining the paperboard's recyclability. These recyclable barrier materials form a continuous film that covers the paper or paper board and gives it the required properties for demanding packaging applications. The water-based barrier coatings are generally comprised of an anionic latex and optionally a pigment. The most widely used water-based latexes are styrene butadiene latex and styrene acrylate latex. The most widely used pigments are kaolin clay, ground calcium carbonate, talc, and mica. Examples of water-based latex barrier coatings are readily available from Michelman Inc., Cincinnati, Ohio and Spectra-Kote, Gettysburg, Pa. These recyclable functional polymer coatings still require additional processing and are expensive relative to the cost of untreated paperboard.

For many demanding food packaging and other demanding applications, at least two layers of functional barrier top coating must be applied, further increasing the cost of the final product. Subsequent coatings are necessary to eliminate pinholes and to increase the overall strength and performance of the paperboard. It is well known in the industry that an inexpensive and less functional base coat may be applied to reduce both the overall porosity of the paperboard and the amount of functional top coat required. The most commonly used base coats include, but are not limited to, kaolin clay, talc, or calcined clay modified with a latex binder, such as modified styrene butadiene, styrene-acrylate, and polyurethane latexes. For example, a base coat of kaolin clay and styrene-butadiene latex requires a coating weight of between 9 to 27 g/m<sup>2</sup> to improve the Cobb sizing of a functional top coat of Popil.

Cationic pigments are also well-known in the industry and are known to give improved properties over the same pigment in anionic form. In the industry, most cationic wet strength resin treated pigments have been treated at a resin addition level of less than 10%, based on the dry weight of the pigment. Generally, these coatings have been used as top coats. There is, however, still a need in the industry for cost-effective ways to provide a paperboard product for processes that require highly resistant barrier properties.

Water-based pigment coatings are also often added to one or both side of paper or paper board to improve the appearance of the paper or paper board, or to improve print quality. As an example, No. 5 ground-wood containing, light weight coated offset sheet is coated with a blend of kaolin/GCC/latex which provides 70% brightness, 50% of gloss, and a Parker Print Surf smoothness of 1.20. Water-based pigment coatings are generally comprised of a pigment or mixture of anionic pigments, and an anionic latex binder. The most widely used pigments are kaolin clay, ground calcium carbonate, and titanium dioxide. The most widely used synthetic binders are styrene butadiene (SB) latex and styrene acrylate (SA) latex. Examples of some commonly used SB latex include Dow RAP316, Dow 620, BASF Styronal 4681 and SA latex, BASF Acronal S504. In demanding applications two to three layers of pigment coating are needed to obtain the desired appearance and print quality. There is also a need to reduce the number of coating steps and the amount of pigment coating needed to obtain the desired appearance and print quality.

**BRIEF SUMMARY OF THE INVENTION**

The present invention relates, in general, to the surprising discovery that a significantly increased addition of cationic wet strength polymer resins to anionic pigments can create a dispersion for use in coating processes that has superior barrier properties when used as a base coating for paper or paper board. This discovery allows for the cost-effective production of highly resistant paperboard for applications that require durability and high barrier resistance to liquid water, water vapor, gas permeability, oil and grease, slip, and static. The discovery also allows for the production of pigment coated paper or paper board with improved appearance and print quality. The present invention also relates to a novel method of improving the performance and reducing the cost of paper and paperboard by using the cationic pigment dispersion as the base coat underneath a functional barrier coating or pigment coating top layer.

One embodiment of the present invention includes a method for increasing one or more barrier properties of a sheet of paper or paperboard, comprising: coating at least one side of the sheet of paper or paperboard with a dispersion having a cationic zeta potential comprising (1) a mixture containing one or more anionic pigments with (2) one or more polyamine-epihalohydrin cationic wet strength resins at a coating weight of from about 0.1 g/m<sup>2</sup> to about 20 g/m<sup>2</sup>; drying the coated sheet of paper or paperboard; and coating the dried sheet of paper or paperboard with a latex based functional barrier top coating formulated to provide resistance to one or more of the following (1) liquid water, (2) water vapor, (3) food oils, (4) grease, (5) gas permeability, (6) skid, or (7) static.

A second embodiment of the present invention includes a method for improving the appearance or printability of a sheet of paper or paperboard, comprising: coating at least one side of the sheet of paper or paperboard with a dispersion having a cationic zeta potential comprising (1) a mixture containing one or more anionic pigments with (2) one or more polyamine-epihalohydrin cationic wet strength resins at a coating weight of from about 0.1 g/m<sup>2</sup> to about 20 g/m<sup>2</sup>; drying the coated sheet of paper or paperboard; and coating the dried sheet of paper or paperboard with a water based pigment coating.

Another embodiment of the invention is a dispersion having a cationic zeta potential for use as a base coating on a sheet of paper or paperboard as a primer for a functional

barrier top coating, comprising: (a) one or more anionic pigments in an amount of at least about 20% dry weight of the anionic pigment-containing mixture, and (b) one or more polyamine-epihalohydrin cationic wet strength resins as well as paper or paperboard coated with this dispersion.

#### DETAILED DESCRIPTION OF THE INVENTION

As used herein, the singular terms "a" and "the" are synonymous and used interchangeably with "one or more" or "at least one" unless the context clearly indicates a contrary meaning. Accordingly, for example, reference to "a compound" herein or in the appended claims can refer to a single compound or more than one compound. Additionally, all numerical values, unless otherwise specifically noted, are understood to be modified by the word "about." Unless otherwise indicated, the terms "dry weight %" and "% dry weight" mean the dry weight percent of the mixture containing only the anionically charged pigment and the optional water soluble polymer binder, and exclude the weight of the polyamine-epihalohydrin cationic wet strength resin. Unless otherwise indicated, all ratios are weight ratios between the cationic resin and the anionic pigment, and exclude the weight of any optional water soluble binder.

Compositions and processes in accordance with the various embodiments of the present invention are suitable for use to coat a sheet of paper or paperboard to increase its barrier resistant properties or improve its appearance or print quality. The present invention includes a novel dispersion composition of anionic pigment, polyamine-epihalohydrin cationic wet strength resin, and an optional neutral or cationic, natural or synthetic polymer binder. The present invention also includes a method of improving the performance and reducing the cost of manufacturing paper and paper board with high barrier resistance to liquid water, water vapor, gas permeability, oil and grease, slip, and static. The method can also be used to reduce the cost of manufacturing of pigment coated paper or paper board with improved appearance or print quality.

The method comprises three steps: (1) coating paper or paper board with a base coat of a dispersion formed by combining (i) a mixture containing one or more anionically charged pigments and, optionally, one or more water soluble polymer binders with (ii) a polyamine-epihalohydrin cationic wet strength resin; (2) drying the coated paper or paper board; and (3) applying a functional barrier top coating that resists one or more of the following: liquid water, water vapor, gas permeability, oil and grease, slip, and static, or an anionic latex based pigment coating that imparts improved opacity, brightness, or printability.

It is believed that the base coat reduces the porosity of the paper or paper board because the pigments in the dispersion deposit in the natural pores of the paper or paperboard. This reduces the amount of functional barrier top coating needed to obtain the desired barrier resistance properties. Adding the base coat is believed to reduce the amount of pigment coating needed to obtain even, consistent coverage of the paper or paper board. Even coating coverage smoothes the surface of the coated board, improving its appearance and reducing print mottle. This reduces the overall cost of making high barrier resistant or pigment coated paper or paperboard.

The base coat can be added to one or both sides of the base sheet. The functional barrier top coating or pigment coating performance improve as the coating weight of the base coat increases. Preferably, the paper or paperboard is coated with

the dispersion at a coating weight from about 0.1 to about 20 g/m<sup>2</sup> per side. More preferably, the paper or paperboard is coated with the dispersion at a coating weight from about 1 to about 10 g/m<sup>2</sup> per side. Most preferably, the paper or paperboard is coated with the dispersion at a coating weight from about 1.5 to about 5.0 g/m<sup>2</sup> per side. For the above, the coating weight is based on the weight of the dried coating.

The pigment for the dispersion can be any of the synthetic or natural pigments used in papermaking, paper coating, or paint applications. Preferably, the pigment is a talc, kaolin clay, bentonite clay, or laponite. More preferably, the pigment is bentonite clay or talc. Most preferably, the pigment is talc.

The percentage of pigment in the mixture of anionic pigment and water soluble polymeric binder required to obtain the desired improvements in barrier resistance depends on the particle size and aspect ratio of the pigment. In general, when small particle size, high aspect ratio pigments—such as laponite or bentonite clay—are used in the invention, the mixture contains pigment addition levels of at least about 20% dry weight of the mixture (with the bulk of remainder of the mixture being the water soluble polymeric binder) to obtain the desired benefits. Preferably, the mixture contains from about 25% to about 100% dry weight of laponite or bentonite clay. More preferably, when laponite is used as the pigment, the mixture contains from about 25% to about 50% dry weight of laponite. More preferably, when bentonite clay is used as the pigment, the mixture contains from about 25% to about 75% dry weight of bentonite clay and 75% to 25% water soluble polymeric binder.

When large particle size, lower aspect ratio pigments—such as kaolin clay or talc—are used in the invention, then the mixture contains pigment addition levels of at least about 25% dry weight of the mixture to obtain the desired benefits. More preferably, when kaolin clay or talc is used as the pigment, the mixture contains from about 50% to about 100% dry weight of kaolin clay or talc. Most preferably, when kaolin clay or talc is used as the pigment, the mixture contains about 75% dry weight of kaolin clay or talc.

The polyamine-epihalohydrin cationic wet strength resin can be any of the resins widely used to impart temporary or permanent wet strength to paper, liquid packaging board, or paperboard. Examples of these resins are known in the industry as disclosed in U.S. Pat. Nos. 7,081,512; 6,554,961; and 5,668,246, the disclosures of which are incorporated herein by reference. The polyamine-epihalohydrin cationic wet strength resins of the present invention include, but are not limited to, polyaminopolyamide-epihalohydrin resins, such as polyaminoamide-epihalohydrin resins, polyamide-polyamine-epihalohydrin resins, polyaminepolyamide-epihalohydrin resins, aminopolyamide-epihalohydrin resins, polyamide-epihalohydrin resins; polyalkylene polyamine-epihalohydrin; and polyaminourylene-epihalohydrin resins, copolyamide-polyurylene-epichlorohydrin resins; polyamide-polyurylene-epichlorohydrin resins. In a preferred embodiment of the invention, the epihalohydrin is epichlorohydrin. Preferably the polyamine-epihalohydrin cationic wet strength resin is polyaminourylene-epihalohydrin resin, polyaminopolyamide-epihalohydrin resin, polyamine-epihalohydrin resin, or polyalkyldiallylamine-epihalohydrin resin, all available from Hercules Incorporated, Wilmington, Del. More preferably, the cationic wet strength resin is polyaminopolyamide-epihalohydrin resin.

The polyamine-epihalohydrin cationic wet strength resin addition level should be sufficient to reverse the pigment's anionic charge and to give the pigment a cationic (positive)

zeta potential and sufficient to provide a water dispersible coating. The amount of polyamine-epihalohydrin cationic wet strength resin needed to reverse the pigment's anionic charge depends on the charge densities of the cationic resin and the anionic pigment.

When the dispersion contains high charge density, high surface area pigments—like laponite or bentonite clay—polyamine-epihalohydrin cationic wet strength resin:anionic pigment ratios from about 0.5:1 to about 2:1 are preferred. Preferably, when the dispersion contains laponite, polyamine-epihalohydrin cationic wet strength resin:anionic pigment ratios are about 1.5:1. Preferably, when the dispersion contains bentonite clay, polyamine-epihalohydrin cationic wet strength resin:anionic pigment ratios from about 0.6:1 to about 0.8:1 are preferred.

When the dispersion contains low charge density, low surface area pigments—such as kaolin clay or talc—polyamine-epihalohydrin cationic wet strength:anionic pigment ratios from about 0.01:1 to about 0.2:1 are preferred. More preferably, when the dispersion contains kaolin clay or talc, cationic wet strength resin:anionic pigment ratios are from about 0.03:1 to about 0.1:1.

The dispersion optionally contains one or more neutral or cationic, natural or synthetic water soluble polymer binders. These binders are common in the paper industry, and are typically used in wet-end dry strength, size press dry strength, and paper coating co-binder applications. Examples of these polymer binders are disclosed in U.S. Pat. Nos. 6,429,253; 6,359,040; and 6,030,443, the disclosures of which are incorporated herein by reference. The binders increase the strength and physical integrity of the coated paper or paperboard product. Here, the binders may improve adhesion of the base coat to the paperboard, and increase the strength and physical integrity of the base coat itself.

Examples of natural water soluble binders include, but are not limited to, starch; ethylated starch; cationic starch; oxidized starch; enzyme converted starch; alginates; proteins, such as casein; cellulose derivatives, such as hydroxyethylcellulose, methylhydroxyethylcellulose, methyl cellulose, hydroxypropyl cellulose or hydroxypropylguar cellulose; and mixtures thereof. Examples of synthetic water soluble binders include, but are not limited to, polyvinylalcohol; ethylene/vinyl alcohol copolymers; polyvinylamine; polyacrylamide; neutrally and cationically charged copolymers of polyacrylamide; glyoxylated polyacrylamide; polydiallylamine; polydimethylallylamine; and copolymers of polydiallylamine or polydimethylallylamine.

Preferably, dispersions containing polyamine-epihalohydrin cationic wet strength resin modified laponite or bentonite clay are made from an anionic pigment-containing mixture containing from about 0% to about 75% dry weight water soluble polymer binders and from about 25% to about 100% dry weight laponite or bentonite pigment. More preferably, dispersions containing polyamine-epihalohydrin cationic wet strength resin modified laponite are made from an anionic pigment-containing mixture containing from about 50% to about 75% dry weight water soluble polymer binder and from about 25% to about 50% dry weight laponite pigment. Also more preferably, dispersions containing polyamine-epihalohydrin cationic wet strength resin modified bentonite clay are made from an anionic pigment-containing mixture containing from about 25% to about 75% dry weight water soluble polymer binder and from about 25% to about 75% dry weight bentonite clay pigment. For the above, the dry weight percents refer to the dry weight of the anionic pigment-containing mixture and do not include the cationic wet strength resin.

Preferably, dispersions containing polyamine-epihalohydrin cationic wet strength resin modified talc or kaolin clay are made from an anionic pigment-containing mixture containing from about 0% to about 75% dry weight water soluble polymer binder and from about 25% to about 100% dry weight talc or kaolin clay pigment. More preferably, dispersions containing polyamine-epihalohydrin cationic wet strength resin modified talc or kaolin clay are made from an anionic pigment-containing mixture containing from about 25% to about 50% dry weight water soluble polymer binder and from about 50% to about 75% dry weight talc or kaolin clay pigment. For the above, the dry weight percents refer to the dry weight of the anionic pigment-containing mixture and do not include the cationic wet strength resin.

The base coat is applied and dried using equipment common in the industry for the application of surface treatments to paper or paper board. These include, but are not limited to, paper machine size presses; spray bars; water boxes; on-machine coaters; and off-machine coaters.

The functional barrier top coating can be any coating commonly used in the paper industry, such as Vaporcoat 1500 and Vaporcoat 2200, available from Michelman Inc., Cincinnati, Ohio, or Spectra-Guard 763, available from Spectra-Kote, Gettysburg, Pa. The functional barrier top coating contains at least one water-based polymer latex. Optionally, the functional barrier top coating may contain one or more natural or synthetic water soluble polymers, such as starch; ethylated starch; succinic anhydride modified starch; polyvinylalcohol; ethylene/vinylalcohol copolymers; or polylactic acid. Additionally, the functional barrier top coating may also contain one or more pigments, waxes, cross-linkers, water resistant sizing agents, and oil and grease resistant sizing agents.

The pigment coating can be any coating commonly used in the paper industry. Water based pigment coatings are primarily comprised of a pigment, or mixture of pigments, and an anionic polymer latex binder. Typical pigments include: kaolin clay, calcined kaolin clay, titanium dioxide, talc, precipitated calcium carbonate, and ground calcium carbonate. The most widely used latex binders are: styrene/butadiene, styrene acrylate, and polyvinylacetate latexes. Water soluble polymer thickeners and binders such as starch, polyvinylalcohol, hydroxyethylcellulose and carboxymethylcellulose (CMC) are also often included in the pigment coating. Other additives, such as, dispersants, defoamers, preservatives, lubricants, and cross-linkers are also often included in the coating formulation.

As one skilled in the art will recognize, the invention is useful in applications that require a highly functional barrier top coating that is resistant to one or more of the following: liquid water; water vapor; oil and grease; gases; skid; and static. The invention is also useful in demanding coated paper or paper board applications.

## EXAMPLES

For each of the following examples, if the dispersion consists of a water soluble binder, pigment and cationic wet strength resin, the following naming convention is used: XX:YY binder:pigment:resin, where XX is the dry weight % of binder and YY is the dry weight % of the pigment in the anionic pigment containing mixture and excludes the cationic wet strength resin. As previously disclosed, dry weight % is the weight of the binder/pigment mixture and excludes the cationic wet strength resin.

## Preparation of Cationic Polymer Modified Pigments

Samples of cationic polymer modified pigments were prepared by adding various amounts of cationic wet strength resin to anionic pigments. For each sample, Kymene 557 (polyaminopolyamide-epihalohydrin) (1% solids content), available from Hercules Incorporated, Wilmington, Del., was used. In Example 1, the pigment used was delaminated Hydrogloss 90 kaolin clay (0.5 micron median particle size; 96% less than 2 microns), available from J. M. Huber, Macon, Ga. In Example 2, the pigment used was talc (1-2 microns), available from Rio Tinto—Talc de Luzenac, Toulouse Cedex, France. In Example 3, the pigment used was bentonite (200-300 nanometers), available from Southern Clay Products Inc., Gonzalez, Tex. In Example 4, the pigment used was Laponite RD (25 nanometers), a synthetic pigment available from Southern Clay Products Inc., Gonzalez, Tex. Each of the pigments was in a 1% solids dispersion.

For each Example, various amounts of Kymene 557 corresponding to a percentage of the dry weight of the pigment were added. After each addition, the zeta potential of each sample was measured. Once the charge on the anionic pigment had reversed, additional Kymene 557 was added to determine the optimal Kymene 557 levels to achieve a well-dispersed pigment dispersion with a mean particle size distribution similar to the anionic pigment dispersions. The results for each Example are listed in Table 1. Unless otherwise noted, the dispersion with an asterisk (\*) is the dispersion referenced in subsequent Examples.

The various Examples show that each of the four anionic pigments begin to floc as its zeta potential approaches 0. Once the pigment reverses charge, however, it begins to re-disperse. The dispersion was considered "well-dispersed" once the dispersion had a mean particle size roughly equivalent to the original anionic pigment dispersion. The amount of polyamine-epihalohydrin resin necessary to achieve this dispersion ranged from approximately 1% of the dry weight of the pigment to approximately 200% of the dry weight of the pigment. In general, pigments with lower charge densities require less polyamine-epihalohydrin resin to reverse the charge and form a well-dispersed cationic pigment.

TABLE 1

## Preparation of Cationic Polymer Modified Pigments

| Example Number | Pigment       | Cationic Polymer | Addition Level (Based on pigment) | Zeta Potential | Comments         |
|----------------|---------------|------------------|-----------------------------------|----------------|------------------|
| 1              | Bentolite H   | —                | —                                 | -35            | Well dispersed   |
|                | Bentolite H   | Kymene 557       | 5.0%                              | -34            | Flocked          |
|                | Bentolite H   | Kymene 557       | 10%                               | -37            | Flocked          |
|                | Bentolite H   | Kymene 557       | 20%                               | +17            | Flocked          |
|                | Bentolite H   | Kymene 557       | 40%                               | +16            | Flocked          |
|                | Bentolite H   | Kymene 557       | 60%                               | +29            | Well dispersed   |
| 2              | Bentolite H   | Kymene 557       | 80%                               | +30            | Well dispersed   |
|                | Hydragloss 90 | —                | —                                 | -34            | Well dispersed   |
| *2             | Hydragloss 90 | Kymene 557       | 1.0%                              | -18            | Flocked          |
|                | Hydragloss 90 | Kymene 557       | 3.0%                              | +20            | Flocked          |
| *3             | Hydragloss 90 | Kymene 557       | 5.0%                              | +81            | Well dispersed   |
|                | Hydragloss 90 | Kymene 557       | 7.0%                              | —              | Well dispersed   |
| 3              | Talc          | —                | —                                 | -28.1          | Well dispersed   |
|                | Talc          | Kymene 557       | 1.0%                              | +12            | Well dispersed   |
|                | Talc          | Kymene 557       | 3.0%                              | +35            | Well dispersed   |
| *4             | Talc          | Kymene 557       | 5.0%                              | +27            | Well dispersed   |
|                | Talc          | Kymene 557       | 10%                               | +29            | Well dispersed   |
|                | Talc          | Kymene 557       | 20%                               | +42            | Well dispersed   |
| 4              | Laponite      | —                | —                                 | -20            | Well dispersed   |
|                | Laponite      | Kymene 557       | 50%                               | +25            | Flocked          |
|                | Laponite      | Kymene 557       | 100%                              | +24            | Slightly flocked |
| *5             | Laponite      | Kymene 557       | 150%                              | +9             | Well dispersed   |

## Preparation of Kymene 557 Modified Talc/Starch Dispersions

Samples of 20% solids Kymene 557 modified talc dispersions for use in size press applications were prepared with varied amounts of starch. For example, to prepare the 25:75 starch:talc:Kymene 557 dispersion, a quantity of 9 g of Vantalc 6H II (0.8-1.3 microns), available from R. T. Vanderbilt, Norwalk, Conn., was dispersed into 36 g of distilled water using an over-head stirrer. A 30% solids solution of Penfordgum 280 ethylated starch, available from Penford, Cedar Rapids, Iowa, was prepared by heating the 10 Penfordgum at between 95 and 100°C. for approximately 45 minutes. A 7.2 g aliquot of Kymene 557H (6.25% solids), available from Hercules Incorporated, Wilmington, Del., was added to 10 g of the cooked starch and mixed. Once the 15 Kymene 557 and starch were well mixed, a quantity of 45 g of the talc dispersion was added and the dispersion was stirred for 5 minutes to create the dispersion. The dispersion was sonicated for 6 minutes using a Branson Sonifier 450 (50% output, setting 4). Finally, the pH of the dispersion was adjusted to 8.0 using NaOH.

Similar methods were used to make the range of starch: 20 pigment:Kymene 557 dispersions listed in Table 2.

## Example 6

## Size Press Base Coat Addition Method

The samples prepared in Example 5 were applied to liner board using a laboratory puddle size press. The Brookfield viscosity of the various Kymene 557 modified laponite, bentonite clay, kaolin clay, and talc dispersions limited their 30 maximum percent solids for size press applications. In order to achieve optimum coating, the Brookfield viscosities of the dispersions, when measured at 100 rpm and 55°C., should be below 200 cps in the size press. For the selected samples a Brookfield viscosity of approximately 100 cps corresponds to approximately 20% solids when the dispersion contains kaolin clay or talc; approximately 5% solids when the 35

dispersion contains bentonite clay; and approximately 3% solids when the dispersion contains laponite.

The samples were applied to individual sheets of 200 g/m<sup>2</sup> (basis weight) 11 cm×28 cm commercial recycled liner board, available from Green Bay Packaging Inc., Green Bay, Wis., using a laboratory puddle size press. Before each run, the size press rolls were heated to 50° C. by allowing hot water to run over the rolls for five minutes. A 100 mL aliquot of each sample was poured into the size press nip, and the recycled liner board sheets were then passed through the nip. The sheets were immediately dried to 5% moisture using a drum dryer set at 220° F. The coating weight of the coated liner board was calculated using the difference in weight of the coated (wet weight) and uncoated sheets. The size press base coat treated sheets were cured at 85° C. for 30 minutes prior to addition of the functional barrier top coating.

#### Example 7

##### Application of Functional Barrier Top Coatings to Paper Board

A 5.1 cm×12.7 cm sheet of polyester was clipped to a standard office clipboard that was duct taped to a lab bench. The reverse side of the sheet was then secured using 2-sided masking tape. A pre-weighed 10.2 cm×16.5 cm sheet of liner board was secured next to the polyester sheet using an exposed edge of the 2-sided masking tape. A bead of functional barrier top coating was applied to the polyester sheet next to the liner board substrate. The functional barrier top coating was applied using a wire-wound drawdown rod pulled through the bead of coating and over the liner board sheet. The coated sheets were allowed to air-dry for one hour, then cured in an oven for two hours at 85° C. The coating weight of the functional barrier top coating applied was determined by comparing the dry weights of the uncoated and coated samples. Coat weight was varied by changing the rod number and varying the % solids of the functional barrier top coating.

#### Example 8

##### Evaluation of Various Starch:Pigment:Kymene 557 Mixtures

Combinations of dispersions containing Kymene 557 modified pigments with starch were evaluated. The pigments used were Vantalc 6HII talc, available from R. T. Vanderbilt, Hydraglass 90 kaolin clay, available from J. M. Huber, bentonite clay, and laponite. The particle sizes for each pigment was the same as previously disclosed. The dispersions were created and applied as a base coat to recycled liner board as defined in the previous examples (See Tables 1, 2).

The dispersions were applied to both sides of the recycled liner board using the method described in Example 6. After drying, the base coat addition levels varied from 1 to 3 g/m<sup>2</sup> per side. The amount of Kymene 557 modified bentonite and laponite base coats that could be added was limited by the % solids and viscosities of the dispersions.

5 A functional barrier top coating consisting of Vaporcoat 2200, available from Michelman Inc., Cincinnati, Ohio, was applied to the felt side of the base coat treated board using the method described in Example 7. Vaporcoat 2200 is a water-based recyclable functional barrier top coating made using a synthetic polymer latex. A series of Vaporcoat 2200 coated control samples was also made by coating untreated liner board base sheet and a size press starch treated base sheet.

10 Each combination of base coat and Vaporcoat 2200 top coat was tested for 30-minute Cobb sizing (TAPPI method T-441) and moisture vapor transmission rate (MVTR, TAPPI method T-448). Moisture vapor transmission rate was measured at room temperature (20-23° C.) and 85% 15 humidity. A saturated aqueous KBr solution was used to control the relative humidity in the test chamber to 85%. Cobb sizing and MVTR test results were based on an average of three measurements.

20 A comparison over a range of Vaporcoat 2200 top coat weights showed that adding a Kymene 557 modified pigment base coat improved functional barrier top coating efficiency in Cobb sizing applications, when compared to the untreated or size press starch treated controls. These results 25 are shown in Table 2. In general, the performance of the base coat/functional top coat combination improved as the percentage of Kymene 557 modified talc or kaolin in the base coat increased from about 25% to about 100% dry weight of the anionic pigment-containing mixture. The best results 30 were obtained at Kymene 557 modified talc levels of from about 75% to about 100% dry weight of the anionic pigment containing mixture in the base coat. For example, without a base coat, a Vaporcoat 2200 coat weight of at least 10 g/m<sup>2</sup> was needed to obtain a 30-minute Cobb sizing value of 40 35 g/m<sup>2</sup>. A Vaporcoat 2200 coat weight of only 4.2 g/m<sup>2</sup> was needed when a 25:75 starch:talc:Kymene 557 base coat was added to the base sheet. The very high surface area Kymene 557 modified bentonite and laponite pigments gave large increases in Vaporcoat 2200 top coat performance at pigment loading as low as 25% to 50% dry weight of the anionic pigment-containing mixture. These results confirm 40 that adding an inexpensive base coat comprised primarily of cationic wet strength resin modified pigment can greatly reduce the amount of expensive functional barrier top coating 45 needed to obtain high levels of water resistance.

A comparison over a range of Vaporcoat 2200 functional top coat weights showed that adding a Kymene 557 modified pigment base coat improved functional barrier top coating efficiency in MVTR applications. These results are 50 shown in Table 2. In general, the performance of the base coat/functional top coat combination improved as the percentage of Kymene 557 modified talc, bentonite, or kaolin in the base coat increased from 25% to 75% dry weight of the anionic pigment-containing mixture. For example, without a 55 base coat, a Vaporcoat 2200 coat weight of 9.8 g/m<sup>2</sup> was needed to obtain a MVTR of 50 g/m<sup>2</sup>/day. A Vaporcoat 2200 coat weight of only 5.5 g/m<sup>2</sup> was needed when a 25:75 starch:talc:Kymene 557 dispersion was added to the base sheet. The best results were obtained when Kymene 557 60 modified talc comprised 75% to 100% dry weight of the anionic pigment-containing mixture of the base coat formulation. A Vaporcoat 2200 coat weight of 5.3 g/m<sup>2</sup> was needed to obtain a MVTR of 50 g/m<sup>2</sup>/day when a 25:75 starch:bentonite:Kymene 557 dispersion was added to the base sheet. The Kymene 557 modified kaolin clay and laponite 65 base coats also gave significant improvements in functional barrier top coating MVTR efficiency.

TABLE 2

|     |                                       | Evaluation of various dispersions                    |                                                     |                                          |                                 |
|-----|---------------------------------------|------------------------------------------------------|-----------------------------------------------------|------------------------------------------|---------------------------------|
| Run | Size Press<br>Base Coat               | Base Coat<br>Add'n Level<br>(g/m <sup>2</sup> /side) | Top Coat<br>Add'n Level<br>(g/m <sup>2</sup> /side) | 30-Minute<br>Cobb<br>(g/m <sup>2</sup> ) | MVTR<br>(g/m <sup>2</sup> /day) |
| 1   | Blank                                 | 0                                                    | 0                                                   | 82                                       | —                               |
| 2   | Blank                                 | 0                                                    | 4.0                                                 | 62                                       | 255                             |
| 3   | Blank                                 | 0                                                    | 7.8                                                 | 61                                       | 199                             |
| 4   | Blank                                 | 0                                                    | 9.8                                                 | 50                                       | 51                              |
| 5   | Blank                                 | 0                                                    | 10.6                                                | 33                                       | —                               |
| 6   | Starch                                | 2.8                                                  | 0                                                   | 120                                      | —                               |
| 7   | Starch                                | 2.8                                                  | 4.2                                                 | 80                                       | 220                             |
| 8   | Starch                                | 2.8                                                  | 6.6                                                 | 75                                       | 148                             |
| 9   | Starch                                | 2.8                                                  | 8.1                                                 | 59                                       | 79                              |
| 10  | 75:25 Starch:Talc:Kymene 557          | 2.8                                                  | 0                                                   | 93                                       | —                               |
| 11  | 75:25 Starch:Talc:Kymene 557          | 2.8                                                  | 3.8                                                 | 71                                       | 174                             |
| 12  | 75:25 Starch:Talc:Kymene 557          | 2.8                                                  | 5.4                                                 | 66                                       | 111                             |
| 13  | 75:25 Starch:Talc:Kymene 557          | 2.8                                                  | 9.1                                                 | 49                                       | 57                              |
| 14  | 50:50 Starch:Talc:Kymene 557          | 2.7                                                  | 0                                                   | 79                                       | —                               |
| 15  | 50:50 Starch:Talc:Kymene 557          | 2.7                                                  | 3.8                                                 | 63                                       | 186                             |
| 16  | 50:50 Starch:Talc:Kymene 557          | 2.7                                                  | 6.4                                                 | 49                                       | 67                              |
| 17  | 25:75 Starch:Talc:Kymene 557          | 2.4                                                  | 0                                                   | 72                                       | —                               |
| 18  | 25:75 Starch:Talc:Kymene 557          | 2.4                                                  | 1.5                                                 | 47                                       | 193                             |
| 19  | 25:75 Starch:Talc:Kymene 557          | 2.4                                                  | 4.2                                                 | 37                                       | 94                              |
| 20  | 25:75 Starch:Talc:Kymene 557          | 2.4                                                  | 5.5                                                 | 12                                       | 32                              |
| 21  | 0:100 Starch:Talc:Kymene 557          | 2.1                                                  | 0                                                   | 63                                       | —                               |
| 22  | 0:100 Starch:Talc:Kymene 557          | 2.1                                                  | 0.5                                                 | 50                                       | 234                             |
| 23  | 0:100 Starch:Talc:Kymene 557          | 2.1                                                  | 2.3                                                 | 36                                       | 139                             |
| 24  | 0:100 Starch:Talc:Kymene 557          | 2.1                                                  | 4.8                                                 | 9                                        | 55                              |
| 25  | 75:25 Starch:Laponite:Kymene 557      | 1.0                                                  | 0                                                   | 69                                       | —                               |
| 26  | 75:25 Starch:Laponite:Kymene 557      | 1.0                                                  | 2.5                                                 | 38                                       | 222                             |
| 27  | 75:25 Starch:Laponite:Kymene 557      | 1.0                                                  | 5.1                                                 | 32                                       | 127                             |
| 28  | 75:25 Starch:Laponite:Kymene 557      | 1.0                                                  | 5.5                                                 | 14                                       | 67                              |
| 29  | 65:35 Starch:Laponite:Kymene 557      | 1.1                                                  | 0                                                   | 64                                       | —                               |
| 30  | 65:35 Starch:Laponite:Kymene 557      | 1.1                                                  | 5.6                                                 | 35                                       | 204                             |
| 31  | 65:35 Starch:Laponite:Kymene 557      | 1.1                                                  | 5.9                                                 | 28                                       | 89                              |
| 32  | 65:35 Starch:Laponite:Kymene 557      | 1.1                                                  | 7.5                                                 | 12                                       | 46                              |
| 33  | 75:25 Starch:Hydragloss 90:Kymene 557 | 2.9                                                  | 0                                                   | 85                                       | —                               |
| 34  | 75:25 Starch:Hydragloss 90:Kymene 557 | 2.9                                                  | 7.3                                                 | 68                                       | 183                             |
| 35  | 75:25 Starch:Hydragloss 90:Kymene 557 | 2.9                                                  | 8.2                                                 | 49                                       | 111                             |
| 36  | 50:50 Starch:Hydragloss 90:Kymene 557 | 2.7                                                  | 0                                                   | 83                                       | —                               |
| 37  | 50:50 Starch:Hydragloss 90:Kymene 557 | 2.7                                                  | 6.1                                                 | 62                                       | 200                             |
| 38  | 50:50 Starch:Hydragloss 90:Kymene 557 | 2.7                                                  | 7.9                                                 | 44                                       | 102                             |
| 39  | 25:75 Starch:Hydragloss 90:Kymene 557 | 2.5                                                  | 0                                                   | 84                                       | —                               |
| 40  | 25:75 Starch:Hydragloss 90:Kymene 557 | 2.5                                                  | 4.5                                                 | 53                                       | 178                             |
| 41  | 25:75 Starch:Hydragloss 90:Kymene 557 | 2.5                                                  | 6.9                                                 | 24                                       | 57                              |
| 42  | 0:100 Starch:Hydragloss 90:Kymene 557 | 2.1                                                  | 0                                                   | 85                                       | —                               |
| 43  | 0:100 Starch:Hydragloss 90:Kymene 557 | 2.1                                                  | 2.7                                                 | 53                                       | 262                             |
| 44  | 0:100 Starch:Hydragloss 90:Kymene 557 | 2.1                                                  | 6.5                                                 | 42                                       | 148                             |
| 45  | 0:100 Starch:Hydragloss 90:Kymene 557 | 2.1                                                  | 8.5                                                 | 18                                       | 53                              |
| 46  | 50:50 Starch:Bentonite:Kymene 557     | 1.6                                                  | 0                                                   | 72                                       | —                               |
| 47  | 50:50 Starch:Bentonite:Kymene 557     | 1.6                                                  | 5.8                                                 | 47                                       | 229                             |
| 48  | 50:50 Starch:Bentonite:Kymene 557     | 1.6                                                  | 8.1                                                 | 40                                       | 134                             |
| 49  | 50:50 Starch:Bentonite:Kymene 557     | 1.6                                                  | 8.3                                                 | 28                                       | 80                              |
| 50  | 25:75 Starch:Bentonite:Kymene 557     | 1.6                                                  | 0                                                   | 71                                       | —                               |
| 51  | 25:75 Starch:Bentonite:Kymene 557     | 1.6                                                  | 1.4                                                 | 45                                       | 222                             |
| 52  | 25:75 Starch:Bentonite:Kymene 557     | 1.6                                                  | 5.0                                                 | 32                                       | 125                             |
| 53  | 25:75 Starch:Bentonite:Kymene 557     | 1.6                                                  | 5.3                                                 | 22                                       | 56                              |
| 54  | 0:100 Starch:Bentonite:Kymene 557     | 1.5                                                  | 0                                                   | 69                                       | —                               |
| 55  | 0:100 Starch:Bentonite:Kymene 557     | 1.5                                                  | 4.2                                                 | 46                                       | 251                             |
| 56  | 0:100 Starch:Bentonite:Kymene 557     | 1.5                                                  | 5.7                                                 | 40                                       | 175                             |
| 57  | 0:100 Starch:Bentonite:Kymene 557     | 1.5                                                  | 7.5                                                 | 26                                       | 97                              |

## Example 9

## Evaluation of Various Pigments with and without Kymene 557 Modification

Starch:pigment base coats made with unmodified talc, bentonite, and laponite pigments were tested over a recycled liner board base sheet. Penfordgum 280 ethylated starch was used for the evaluation. The percentages of unmodified pigment used in the base coat formulations were selected based on the results described in Example 8. The results are disclosed in Table 3. 50:50 and 25:75 starch:talc:Kymene 557 dispersions were made and evaluated for comparison.

<sup>55</sup> The dispersions were made and applied using the methods described in Examples 5 and 6. The dispersions were applied to both sides of the linerboard. Base coat addition levels varied from 1-3 g/m<sup>2</sup> per side. A Vaporcoat 2200 functional barrier top coating was applied to the felt side of the base coat treated board using the method described in Example 7. A series of Vaporcoat 2200 coated control samples was also made by coating the untreated base sheet.

Each combination of base coat and Vaporcoat 2200 top coat was tested for 30-minute Cobb sizing (TAPPI method T-441) and moisture vapor transmission rate (TAPPI method T-448). Moisture vapor transmission rate was measured at

## 13

room temperature (20-23° C.) and 85% humidity. A saturated aqueous KBr solution was used to control the relative humidity in the test chamber to 85%. Cobb sizing and MVTR test results were based on an average of three measurements.

A comparison at equal Vaporcoat 2200 top coat weights showed that adding a base coat made with unmodified talc or bentonite had little or no beneficial effect on the 30-minute Cobb or MVTR efficiency of the Vaporcoat 2200 functional barrier top coating when compared to the untreated liner board controls. The results are disclosed in Table 3. One of the unmodified laponite base coats gave small improvements in functional barrier top coating efficiency (65:35 starch:laponite). The improvements were smaller than those obtained with base coats made using Kymene 557 modified laponite. Both base coats made with Kymene 557 modified talc gave significant increases in the 30-minute Cobb and MVTR efficiency of the Vaporcoat 2200 top coat.

## 14

described in Table 4. A Vaporcoat 2200 functional barrier top coating, available from Michelman Inc., was applied to both sides of the dispersion treated board. A series of Vaporcoat 2200 coated control samples was also made by coating the untreated base sheet.

Each combination of base coat and Vaporcoat 2200 top coat was tested for 30-minute Cobb sizing (TAPPI method T-441), Kit oil and grease resistance (TAPPI method T-559), and moisture vapor transmission rate (TAPPI method T-448). Moisture vapor transmission rate was measured at room temperature (20-23° C.) and 85% humidity. A saturated aqueous KBr solution was used to control the relative humidity in the test chamber to 85%. Cobb sizing, Kit oil and grease resistance, and MVTR test results were based on an average of three measurements. The results of this testing are shown in Table 4.

A Vaporcoat 2200 functional top coat weight of more than 10 g/m<sup>2</sup> was needed to obtain a 30-minute Cobb sizing value

TABLE 3

| Evaluation of various pigments with and without Kymene 557 |                              |           |                                                |                                               |                                    |                              |
|------------------------------------------------------------|------------------------------|-----------|------------------------------------------------|-----------------------------------------------|------------------------------------|------------------------------|
| Run                                                        | Size Press                   | Base Coat | Base Coat Add'n Level (g/m <sup>2</sup> /side) | Top Coat Add'n Level (g/m <sup>2</sup> /side) | 30-Minute Cobb (g/m <sup>2</sup> ) | MVTR (g/m <sup>2</sup> /day) |
| 1                                                          | Blank                        |           | 0                                              | 0                                             | 240                                | —                            |
| 2                                                          | Blank                        |           | 0                                              | 3.8                                           | 87                                 | 264                          |
| 3                                                          | Blank                        |           | 0                                              | 4.7                                           | 68                                 | 228                          |
| 4                                                          | Blank                        |           | 0                                              | 6.8                                           | 68                                 | 131                          |
| 5                                                          | 50:50 Starch:Talc:Kymene 557 |           | 2.7                                            | 0                                             | 166                                | —                            |
| 6                                                          | 50:50 Starch:Talc:Kymene 557 |           | 2.7                                            | 2.6                                           | 72                                 | 196                          |
| 7                                                          | 50:50 Starch:Talc:Kymene 557 |           | 2.7                                            | 2.9                                           | 62                                 | 143                          |
| 8                                                          | 50:50 Starch:Talc:Kymene 557 |           | 2.7                                            | 4.0                                           | 49                                 | 89                           |
| 9                                                          | 25:75 Starch:Talc:Kymene 557 |           | 2.4                                            | 0                                             | 194                                | —                            |
| 10                                                         | 25:75 Starch:Talc:Kymene 557 |           | 2.4                                            | 0.5                                           | 57                                 | 227                          |
| 11                                                         | 25:75 Starch:Talc:Kymene 557 |           | 2.4                                            | 4.2                                           | 29                                 | 62                           |
| 12                                                         | 50:50 Starch:Talc            |           | 2.7                                            | 0                                             | 195                                | —                            |
| 13                                                         | 50:50 Starch:Talc            |           | 2.7                                            | 4.0                                           | 106                                | 217                          |
| 14                                                         | 50:50 Starch:Talc            |           | 2.7                                            | 5.1                                           | 72                                 | 150                          |
| 15                                                         | 25:75 Starch:Talc            |           | 2.6                                            | 0                                             | 204                                | —                            |
| 16                                                         | 25:75 Starch:Talc            |           | 2.6                                            | 4.6                                           | 77                                 | 239                          |
| 17                                                         | 25:75 Starch:Talc            |           | 2.6                                            | 5.6                                           | 70                                 | 184                          |
| 18                                                         | 25:75 Starch:Talc            |           | 2.6                                            | 8.4                                           | 61                                 | 117                          |
| 19                                                         | 75:25 Starch:Laponite        |           | 1.2                                            | 0                                             | 167                                | —                            |
| 20                                                         | 75:25 Starch:Laponite        |           | 1.2                                            | 5.2                                           | 66                                 | 235                          |
| 21                                                         | 75:25 Starch:Laponite        |           | 1.2                                            | 10.6                                          | 61                                 | 117                          |
| 22                                                         | 65:35 Starch:Laponite        |           | 1.0                                            | 0                                             | 150                                | —                            |
| 23                                                         | 65:35 Starch:Laponite        |           | 1.0                                            | 2.7                                           | 56                                 | 242                          |
| 24                                                         | 65:35 Starch:Laponite        |           | 1.0                                            | 5.7                                           | 50                                 | 142                          |
| 25                                                         | 50:50 Starch:Bentonite       |           | 1.6                                            | 0                                             | 217                                | —                            |
| 26                                                         | 50:50 Starch:Bentonite       |           | 1.6                                            | 3.6                                           | 81                                 | 229                          |
| 27                                                         | 50:50 Starch:Bentonite       |           | 1.6                                            | 6.1                                           | 72                                 | 163                          |
| 28                                                         | 25:75 Starch:Bentonite       |           | 1.5                                            | 0                                             | 238                                | —                            |
| 29                                                         | 25:75 Starch:Bentonite       |           | 1.5                                            | 4.4                                           | 73                                 | 231                          |
| 30                                                         | 25:75 Starch:Bentonite       |           | 1.5                                            | 11.1                                          | 63                                 | 127                          |

## Example 10

## Effect of Base Coat Coating Weight on Barrier Resistance

A base coat made from a dispersion of 25:75 Penfordgum 280 ethylated starch:talc:Kymene 557 was evaluated at three size press coating weights. A base coat made from a 25:75 mixture of Prequel 500 cationic starch, available from Hercules Incorporated, Wilmington, Del., and Kymene 557 modified talc was tested at two coating weights.

The dispersions were made and applied to recycled liner board using the methods described in Examples 5 and 6. The dispersion was applied to both sides of the liner board. Coating weights varied from 1.5-4.5 g/m<sup>2</sup> per side as

below 20 g/m<sup>2</sup> over the untreated liner board control. A Vaporcoat 2200 functional top coat weight of 7.1 g/m<sup>2</sup> was needed to obtain the same level of Cobb sizing over either of the Kymene 557 modified talc base coats. In both cases, size press base coat addition levels of 1.5-2.5 g/m<sup>2</sup> per side gave clear improvements in top coat Cobb sizing efficiency. These results show that a Kymene 557 modified talc base coat made with either ethylated or cationic starch greatly reduces the amount of expensive functional barrier top coating needed for applications that require high levels of water resistance.

Additionally, a Vaporcoat 2200 top coat weight of more than 10 g/m<sup>2</sup> was needed to obtain a MVTR of 34 g/m<sup>2</sup>/day over the untreated base sheet control. Both of the Kymene 557 modified talc base coats significantly improved the

## 15

MVTR efficiency of the Vaporcoat 2200 functional top coat. In both cases, a Vaporcoat 2200 coat weight of 7-8 g/m<sup>2</sup> was needed to obtain the same level of moisture vapor resistance. Size press base coat addition levels of 1.5-2.5 g/m<sup>2</sup> per side were needed to obtain the improved MVTR efficiency.

Finally, a Vaporcoat 2200 functional top coat weight of 12.5 g/m<sup>2</sup> was needed to obtain a Kit oil and grease resistance value of 6 over the untreated liner board control. Both of the Kymene 557 modified talc base coats significantly improved the oil and grease resistance efficiency of the Vaporcoat 2200 top coat. A Vaporcoat 2200 top coat weight of 7-8 g/m<sup>2</sup> was needed to obtain the same level of oil and grease resistance over the Kymene 557 modified talc base coat treated board. Both base coats gave clear improvements in top coat efficiency at addition levels of 1.5-3.5 g/m<sup>2</sup> per side.

TABLE 4

| Evaluation of base coats made with ethylated and cationic starch |                                   |                                                |                                               |                                    |                              |         |
|------------------------------------------------------------------|-----------------------------------|------------------------------------------------|-----------------------------------------------|------------------------------------|------------------------------|---------|
| Size Press Run                                                   | Base Coat                         | Base Coat Add'n Level (g/m <sup>2</sup> /side) | Top Coat Add'n Level (g/m <sup>2</sup> /side) | 30-Minute Cobb (g/m <sup>2</sup> ) | MVTR (g/m <sup>2</sup> /day) | Kit OGR |
| 1                                                                | Blank                             | 0                                              | 5.3                                           | 63                                 | 63                           | 4       |
| 2                                                                | Blank                             | 0                                              | 10.1                                          | 27                                 | 34                           | 4.5     |
| 3                                                                | Blank                             | 0                                              | 12.5                                          | 8                                  | 22                           | 6       |
| 4                                                                | 25:75 Penford 280:Talc:Kymene 557 | 4.3                                            | 8.0                                           | 11                                 | 31                           | 7       |
| 5                                                                | 25:75 Penford 280:Talc:Kymene 557 | 4.3                                            | 9.7                                           | 4                                  | 17                           | 8       |
| 6                                                                | 25:75 Penford 280:Talc:Kymene 557 | 2.6                                            | 7.1                                           | 12                                 | 26                           | —       |
| 7                                                                | 25:75 Penford 280:Talc:Kymene 557 | 2.6                                            | 9.1                                           | 6                                  | 21                           | —       |
| 8                                                                | 25:75 Penford 280:Talc:Kymene 557 | 1.4                                            | 7.2                                           | 17                                 | 32                           | —       |
| 9                                                                | 25:75 Penford 280:Talc:Kymene 557 | 1.4                                            | 9.3                                           | 6                                  | 22                           | —       |
| 10                                                               | 25:75 Prequel 500:Talc:Kymene 557 | 3.5                                            | 7.2                                           | 13                                 | 25                           | 6.7     |
| 11                                                               | 25:75 Prequel 500:Talc:Kymene 557 | 3.5                                            | 10.8                                          | 4                                  | 19                           | 7       |
| 12                                                               | 25:75 Prequel 500:Talc:Kymene 557 | 1.5                                            | 7.5                                           | 9                                  | 31                           | —       |
| 13                                                               | 25:75 Prequel 500:Talc:Kymene 557 | 1.5                                            | 10.0                                          | 6                                  | 32                           | —       |

## Example 11

## Effect of Kymene 557 Addition Level on Talc Performance

Base coats made from dispersions of 25:75 Penfordgum 280 ethylated starch:talc:Kymene 557 were evaluated at Kymene 557 ratios of Kymene 557:talc of 0:1, 0.5:1, and 0.1:1. The results of the evaluation are disclosed in Table 5. The dispersions were made using the method described in Example 5. The effect of adding Kymene 557 (no talc) to the surface of the liner board was also tested. The base coats and Kymene 557 size press treatments were applied to recycled

## 16

liner board using the method described in Example 6. The base coats and Kymene 557 treatments were applied to both sides of the liner board.

A Vaporcoat 2200 functional barrier top coating, available from Michelman Inc. was applied to the felt side of the treated liner board using the method described in Example 7. A series of Vaporcoat 2200 coated control samples was also made by coating the untreated base sheet. Each combination of base coat and Vaporcoat 2200 functional top coat was tested for 30-minute Cobb sizing.

A comparison over a range of coat weights showed that adding a base coat made from a mixture of 25:75 Penford 280 ethylated starch:talc, with no Kymene 557 addition, gave at most small improvements in the Cobb sizing efficiency of the Vaporcoat 2200 top coat. The base coats made

with 0.05:1 and 0.1:1 Kymene 557:talc ratios gave larger improvements in functional barrier top coating efficiency. The base coats made at 0.05:1 and 0.1:1 Kymene 557:talc ratios talc gave similar improvements in top coat efficiency.

Adding Kymene 557 directly to the surface of the liner board gave small improvements in the Cobb sizing efficiency of the Vaporcoat 2200 functional barrier top coating. Both addition levels—0.14% and 0.27%—gave similar improvements in top coat efficiency. The results are disclosed in Table 5. These results show that the combination of Kymene 557 cationic wet strength resin and anionic pigment results in much larger improvements in functional barrier top coating performance than using either Kymene 557 or an anionic pigment separately.

TABLE 5

| Effect of Kymene 557 addition level |                                             |                                                |                                               |                                    |    |  |
|-------------------------------------|---------------------------------------------|------------------------------------------------|-----------------------------------------------|------------------------------------|----|--|
| Size Press Run                      | Base Coat                                   | Base Coat Add'n Level (g/m <sup>2</sup> /side) | Top Coat Add'n Level (g/m <sup>2</sup> /side) | 30-Minute Cobb (g/m <sup>2</sup> ) |    |  |
| 1                                   | Blank                                       | 0                                              |                                               | 6.7                                | 72 |  |
| 2                                   | Blank                                       | 0                                              |                                               | 8.4                                | 71 |  |
| 3                                   | 25:75 Penford 280:Talc:Kymene 557 (1:0)*    | 4.0                                            |                                               | 0.5                                | 94 |  |
| 4                                   | 25:75 Penford 280:Talc:Kymene 557 (1:0)*    | 4.0                                            |                                               | 3.0                                | 78 |  |
| 5                                   | 25:75 Penford 280:Talc:Kymene 557 (1:0)*    | 4.0                                            |                                               | 4.5                                | 65 |  |
| 6                                   | 25:75 Penford 280:Talc:Kymene 557 (1:0.05)* | 4.3                                            |                                               | 1.1                                | 63 |  |
| 7                                   | 25:75 Penford 280:Talc:Kymene 557 (1:0.05)* | 4.3                                            |                                               | 2.1                                | 55 |  |
| 8                                   | 25:75 Penford 280:Talc:Kymene 557 (1:0.05)* | 4.3                                            |                                               | 4.3                                | 31 |  |

TABLE 5-continued

|     |                                            | Effect of Kymene 557 addition level                  |                                                     |                                          |
|-----|--------------------------------------------|------------------------------------------------------|-----------------------------------------------------|------------------------------------------|
| Run | Size Press<br>Base Coat                    | Base Coat<br>Add'n Level<br>(g/m <sup>2</sup> /side) | Top Coat<br>Add'n Level<br>(g/m <sup>2</sup> /side) | 30-Minute<br>Cobb<br>(g/m <sup>2</sup> ) |
| 9   | 25:75 Penford 280:Talc:Kymene 557 (1:0.1)* | 4.0                                                  | 3.3                                                 | 54                                       |
| 10  | 25:75 Penford 280:Talc:Kymene 557 (1:0.1)* | 4.0                                                  | 6.6                                                 | 29                                       |
| 11  | Kymene 557                                 | 0.14% (1x)                                           | 2.7                                                 | 64                                       |
| 12  | Kymene 557                                 | 0.14% (1x)                                           | 4.6                                                 | 55                                       |
| 13  | Kymene 557                                 | 0.14% (1x)                                           | 6.8                                                 | 47                                       |
| 14  | Kymene 557                                 | 0.27% (2x)                                           | 2.9                                                 | 63                                       |
| 15  | Kymene 557                                 | 0.27% (2x)                                           | 4.6                                                 | 46                                       |

\*The ratio in parentheses represents anionic pigment:resin.

15

## Example 12

## Evaluation of Kymene 450, Kymene 736, and Kymene 2064 Modified Talc Base Coats

Base coats made from dispersions of 25:75 Penfordgum 280 ethylated starch:talc:cationic wet strength resin were evaluated where the cationic wet strength resins were Kymene 450, Kymene 736, and Kymene 2064, all available from Hercules Incorporated, Wilmington, Del. The cationic wet strength resin was added at a resin:talc weight ratio of 0.05:1 for each dispersion. The dispersions were made using the method disclosed in Example 5.

Each base coat was evaluated for its effect on the performance of a Vaporcoat 2200 functional barrier top coating. Each base coat was applied to both sides of a sheet of recycled liner board using the method described in Example 6 and a Vaporcoat 2200 functional barrier top coating was applied to the felt side of the treated liner board using the method described in Example 7. A series of liner board samples coated with only the Vaporcoat 2200 functional barrier top coating was used as controls. Each combination of the base coat and Vaporcoat 2200 functional barrier top coating was tested for 30-minute Cobb sizing. The results are disclosed in Table 6.

A comparison over a range of coat weights showed that all three wet strength resin modified talcs improved the Cobb sizing efficiency of the Vaporcoat 2200 functional barrier top coating (versus top coat addition to the untreated base sheet control).

## Example 13

## Evaluation of Kymene 557 Modified Talc Using Polyvinylalcohol as the Binder

20

A base coat was made using a dispersion of 25:75 binder:talc:Kymene 557. The water soluble binder was a 50:50 mixture of Penford 280 ethylated starch:Elvanol 90-50 polyvinylalcohol. The Elvanol 90-50 polyvinylalcohol is available from DuPont, Wilmington, Del. The base coat was made using the method disclosed in Example 5.

Each base coat was evaluated for its effect on the performance of a Vaporcoat 2200 functional barrier top coating. 30 Each base coat was applied to both sides of a sheet of recycled liner board using the method described in Example 6 and a Vaporcoat 2200 functional barrier top coating was applied to the felt side of the treated liner board using the method described in Example 7. A series of liner board samples coated with only the Vaporcoat 2200 function 35 barrier top coating was used as a control. Each combination of the base coat and Vaporcoat 2200 functional barrier top coating was tested for 30-minute Cobb sizing. The results are disclosed in Table 7.

A comparison over a range of coat weights showed that adding the Kymene 557 modified talc base coat improved the Cobb sizing efficiency of the Vaporcoat 2200 functional barrier top coating when a starch:polyvinylalcohol blend was used as the water soluble binder for the base coat.

TABLE 6

|     |                                              | Performance of various wet strength resin modified talcs |                                                     |                                          |
|-----|----------------------------------------------|----------------------------------------------------------|-----------------------------------------------------|------------------------------------------|
| Run | Size Press<br>Base Coat                      | Base Coat<br>Add'n Level<br>(g/m <sup>2</sup> /side)     | Top Coat<br>Add'n Level<br>(g/m <sup>2</sup> /side) | 30-Minute<br>Cobb<br>(g/m <sup>2</sup> ) |
| 1   | Blank                                        | 0                                                        | 2.3                                                 | 86                                       |
| 2   | Blank                                        | 0                                                        | 3.5                                                 | 76                                       |
| 3   | Blank                                        | 0                                                        | 4.4                                                 | 68                                       |
| 4   | Blank                                        | 0                                                        | 5.0                                                 | 66                                       |
| 5   | 25:75 Penford 280:Talc:Kymene 450 (1:0.05)*  | 4.0                                                      | 2.9                                                 | 64                                       |
| 6   | 25:75 Penford 280:Talc:Kymene 450 (1:0.05)*  | 4.0                                                      | 3.3                                                 | 54                                       |
| 7   | 25:75 Penford 280:Talc:Kymene 450 (1:0.05)*  | 4.0                                                      | 3.8                                                 | 39                                       |
| 8   | 25:75 Penford 280:Talc:Kymene 736 (1:0.05)*  | 4.1                                                      | 0.7                                                 | 77                                       |
| 9   | 25:75 Penford 280:Talc:Kymene 736 (1:0.05)*  | 4.1                                                      | 2.2                                                 | 48                                       |
| 10  | 25:75 Penford 280:Talc:Kymene 736 (1:0.05)*  | 4.1                                                      | 4.2                                                 | 33                                       |
| 11  | 25:75 Penford 280:Talc:Kymene 2064 (1:0.05)* | 4.2                                                      | 0.5                                                 | 65                                       |
| 12  | 25:75 Penford 280:Talc:Kymene 2064 (1:0.05)* | 4.2                                                      | 2.3                                                 | 61                                       |
| 13  | 25:75 Penford 280:Talc:Kymene 2064 (1:0.05)* | 4.2                                                      | 3.5                                                 | 44                                       |
| 14  | 25:75 Penford 280:Talc:Kymene 2064 (1:0.05)* | 4.2                                                      | 4.4                                                 | 44                                       |

\*The ratio in parentheses represents anionic pigment:resin.

TABLE 7

Evaluation of Kymene 557 modified talc with 50:50 ethylated starch:polyvinylalcohol water soluble binder

| Run | Size Press<br>Base Coat                            | Base Coat<br>Add'n Level<br>(g/m <sup>2</sup> /side) | Top Coat<br>Add'n Level<br>(g/m <sup>2</sup> /side) | 30-Minute<br>Cobb<br>(g/m <sup>2</sup> ) |
|-----|----------------------------------------------------|------------------------------------------------------|-----------------------------------------------------|------------------------------------------|
| 1   | 12.5:12.5:75 Penford 280:Talc:Kymene 557 (1:0.05)* | 4.5                                                  | 4.6                                                 | 52                                       |
| 2   | 12.5:12.5:75 Penford 280:Talc:Kymene 557 (1:0.05)* | 4.5                                                  | 5.3                                                 | 49                                       |
| 3   | 12.5:12.5:75 Penford 280:Talc:Kymene 557 (1:0.05)* | 4.5                                                  | 6.4                                                 | 45                                       |
| 4   | 50:50 Polyvinylalcohol:Penford 280                 | 5.5                                                  | 4.1                                                 | 105                                      |
| 5   | 50:50 Polyvinylalcohol:Penford 280                 | 5.5                                                  | 5.0                                                 | 109                                      |

\*The ratio in parentheses represents anionic pigment:resin.

#### Example 14

##### Application of Wet Strength Resin Modified Talc and Pigment Coating to Bleached Board

A 20% solids cationic wet strength resin modified talc dispersion was made using the following method. First, 337.5 g of Vantalc 6H II (R. T. Vanderbilt, Norwalk, Conn.) were dispersed into 787.5 g of distilled water using a Cowles mixer (1000 rpm). A 30% solids solution of Penfordgum 280 ethylated starch (112.5 g of starch in 262.5 g of distilled water, Penford, Cedar Rapids, Iowa) was made by cooking at 95-100° C. for 45 minutes. An 834 g aliquot of Kymene 557H (2.0% solids, Hercules, Wilmington, Del.) was then added to 375 g of the cooked starch. The mixture was stirred for 5 minutes using a Cowles blade (1000 rpm). Once the Kymene 557 and starch were well mixed, 1125 g of the talc dispersion were added and stirring was continued for two hours. The pH of the dispersion was adjusted to 8.0 using NaOH.

The Kymene 557 modified talc dispersion was applied to a sample of commercial bleached board (300 g/m<sup>2</sup>) using a Dow bench coater. A control sample was also made by coating the commercial board with a 94:6 mixture of oxidized starch and a styrene/acrylate latex surface sizing agent. In both cases, a wire-wound rod was used to control size press pick-up to 2.2 g/m<sup>2</sup>.

A standard pigment coating was applied to the base coat and starch/latex size press treated board using a cylindrical lab coater (CLC, 460 meters per minute). The coating formulation that was used is listed in Table 1 (67.5% total solids). A metering blade was used to control the amount of coating applied to the board. The coat weights that were obtained are listed in Table 8. A sample of untreated board (no size press treatment) was also coated and tested.

TABLE 8

##### Coating Formulation

100% Ground Calcium Carbonate (GCC) (1.4 micron mean particle size)  
2.6 parts per hundred (pph) starch  
9.9 pph styrene butadiene latex  
0.33 pph polyacrylic acid dispersant  
0.48 pph low viscosity CMC

Coating coverage was used as a measure of the appearance and printability of the coated board. Coating coverage was measured using the burn-out method developed by Dobson (Dobson, R L, "Burnout, a Coat Weight Determination Test Re-Invented." *TAPPI Coating Conference*, pp. 123-131, Chicago, Apr. 21-23, 1975). Increasing coat weight over the untreated blank gave an incremental improvement

15 in coating coverage—70% coverage at 13.8 g/m<sup>2</sup> coat weight versus 67% coverage at 10.2 g/m<sup>2</sup>. When compared at equal pigment coat weight, adding the starch/latex size press treatment did not improve coating coverage—65% coverage at 11.5 g/m<sup>2</sup>. Adding the wet strength resin modified talc size press base coat greatly improved coating coverage versus the Blank. A pigment coating coverage value of 74% was obtained at a coat weight of only 10.8 g/m<sup>2</sup>.

25

TABLE 9

| Pigment Coating Coverage |                   |                      |                                     |                      |
|--------------------------|-------------------|----------------------|-------------------------------------|----------------------|
| Run #                    | S.P. Treatment    | S.P. Pick-up         | Coating Pick-up (g/m <sup>2</sup> ) | Coating Coverage (%) |
| 1                        | Blank             | —                    | 10.2                                | 67                   |
| 2                        | Blank             | —                    | 13.8                                | 70                   |
| 3                        | Starch/Latex      | 2.2 g/m <sup>2</sup> | 11.5                                | 65                   |
| 4                        | WSR Modified Talc | 2.2 g/m <sup>2</sup> | 10.8                                | 74                   |

#### Example 15

##### Application of Wet Strength Resin Modified Talc and Pigment Coating to Light Weight Coated Base Paper

40 A 20% solids cationic wet strength resin modified talc dispersion was made using the method described in Example 14. The dispersion was diluted to 7.4% solids with water then applied to a sample of 33 g/m<sup>2</sup> commercial light weight coated (LWC) base paper using a Dow coater. The talc dispersion coat weight was controlled at 1.0 g/m<sup>2</sup> using a wire-wound rod. The base paper consisted of 60% ground-wood and 40% Kraft pulp. Samples of the base paper pre-coated with Penford PG-280 cooked starch, and a 1/3 blend of PG-280 cooked starch and delaminated clay, were 45 also made. The starch and starch/clay coat weights were controlled at 1.0 g/m<sup>2</sup> using a wire-wound rod.

50 A clay coating was formulated with a blend of 60% delaminated clay (Imerys Astraplate) and 40% No. 2 clay (Huber Hydrasperse), 12 parts of latex (BASF Styronal 4606), and 0.3 parts of thickener (BASF Sterocoll FS). The coating solids and pH were adjusted to 56.7% and 8.3, respectively. Coating color viscosity was 700 cPs as measured by the Brookfield viscometer using 100 rpm and a No. 4 spindle. Using the Dow blade coater, the clay coating was 55 applied onto the pre-coated base papers and a sample of untreated base paper with coat weights controlled at 6.5 g/m<sup>2</sup>.

Coating coverage, opacity, and brightness were used as measures of the appearance and printability of the coated board. The coating coverage of the coated samples was evaluated using the burn-out procedure developed by Dobson. The burn-out image of the sample was assessed for relative coating coverage using an image analyzer. The relative coating coverage results are shown in Table 10. The base paper pre-coated with the wet strength resin modified talc exhibited the highest % coating coverage at equal coat weight. The opacity and brightness of the coated samples are shown in Table 10. The opacity and brightness of the coated paper correlated well with coating coverage. The base paper pre-coated with wet strength resin modified talc exhibited the highest opacity and brightness at equal coated weight.

TABLE 10

| Pigment Coating Coverage, Opacity, and Brightness |                   |                      |                                     |                      |            |
|---------------------------------------------------|-------------------|----------------------|-------------------------------------|----------------------|------------|
| Run #                                             | Pre-treatment     | Pick-up              | Coating Pick-up (g/m <sup>2</sup> ) | Coating Coverage (%) | Brightness |
| 1                                                 | Blank             | —                    | 6.5                                 | 82.9                 | 83.3 69.2  |
| 2                                                 | Starch            | 1.0 g/m <sup>2</sup> | 6.5                                 | 81.2                 | 83.6 70.0  |
| 3                                                 | Starch/Clay       | 1.0 g/m <sup>2</sup> | 6.5                                 | 84.8                 | 84.1 69.8  |
| 4                                                 | WSR Modified Talc | 1.0 g/m <sup>2</sup> | 6.5                                 | 87.5                 | 84.7 70.1  |

It will be appreciated by those skilled in the art that changes could be made to the embodiments described above without departing from the broad inventive concept thereof. It is understood, therefore, that this invention is not limited to the particular embodiments disclosed, but it is intended to cover modifications within the spirit and scope of the present invention as defined by the appended claims.

What is claimed is:

1. A method of coating a sheet of paper or paperboard, comprising:
  - (a) coating at least one side of the sheet of paper or paperboard with a dispersion wherein the dispersion has an overall cationic zeta potential comprising (1) an anionic kaolin clay and/or an anionic talc in an amount of at least about 20% dry weight of the dispersion, and (b) one or more polyaminopolyamide-epihalohydrin resins, wherein the weight ratio of polyaminopolyamide-epihalohydrin resin to anionic clay or talc is from about 0.03:1 to about 0.2:1 and wherein the sheet is coated at a coating weight of from about 0.1 g/m<sup>2</sup> to about 20 g/m<sup>2</sup>; and
  - (b) drying the coated sheet of paper or paperboard.

2. The method claimed in claim 1 further comprising: coating the dried sheet of paper or paperboard with a functional barrier top coating formulated to provide resistance to one or more of the following (1) liquid water, (2) water vapor, (3) oil, (4) grease, (5) gas permeability, (6) skid, or (7) static.

3. The method of claim 2 where the functional barrier top coating contains a water based polymer latex and optionally contains one or more of the following: (1) a natural or synthetic water soluble polymer, (2) a pigment, (3) a wax, (4) a cross-linker, and (5) a sizing agent.

4. The method of claim 3 wherein one or more of the natural or synthetic water soluble polymers is selected from the group consisting of: starch; ethylated starch; oxidized starch; enzyme converted starch; succinic anhydride modified starch; polyvinylalcohol; ethylene/vinylalcohol copolymers; or polylactic acid.

5. The method of claim 2, wherein the functional barrier top coating is applied at a coating weight of not more than about 25 g/m<sup>2</sup>.

20 6. The method claimed in claim 1 further comprising coating the dried sheet of paper or paperboard with a water based pigment coating.

7. The method claimed in claim 6 wherein said water based pigment coating comprises an anionic polymeric latex binder and at least one pigment.

25 8. The method of claim 1 wherein a water soluble binder comprises up to about 80% dry weight of said dispersion, and said binder is selected from the group consisting of: neutral natural water soluble polymer binders; cationic natural water soluble polymer binders; neutral synthetic water soluble polymer binders; and cationic synthetic polymer binders.

30 9. The method of claim 8 wherein the water soluble polymer binder is one or more of the group consisting of: starch; ethylated starch; cationic starch; oxidized starch; enzyme converted starch; alginates; casein; cellulose derivatives; polyvinyl alcohol; ethylene/vinyl alcohol copolymers; polyvinyl amine; polyacrylamide; polyacrylamide copolymers; glyoxylated polyacrylamide; polydiallylamine; polydiallylamine copolymers; polydimethylidiallylamine; and polydimethylidiallylamine copolymers.

35 10. The method of claim 9 wherein the cellulose derivative is one or more of the group consisting of hydroxyethylcellulose; methylhydroxyethylcellulose; methyl cellulose; hydroxypropyl cellulose; and hydroxypropylguar.

40 11. The method of claim 1 wherein said dispersion is at least about 25% dry weight of the dispersion of either anionic kaolin clay or anionic talc.

45 12. The method of claim 1 wherein said dispersion is at least about 50% dry weight of the dispersion of either anionic kaolin clay or anionic talc.

\* \* \* \* \*